

## UNITED STATES PATENT OFFICE

2,662,805

SIMULTANEOUS DRUMMING AND VACUUM  
TREATING OF SKINS

Charles F. Rutherford, Philadelphia, Samuel Cameron Tease, Media, and Harry La Rue Troxell, Jr., Narberth, Pa., assignors to High Vacuum Processes, Inc., Philadelphia, Pa., a corporation of Pennsylvania

No Drawing. Application December 8, 1950,  
Serial No. 199,912

8 Claims. (Cl. 8—12)

1

This invention relates to an apparatus and method for treating leather and skins or producing leather from skins, and more particularly concerns the high vacuum treatment of skins and leather with liquid treating agents.

In conventional operations, pelts such as hides, skins of small animals, and kips, hereinafter generically referred to as skins, are first submerged and soaked in clear water and left for periods up to 48 hours. The cleaned and softened skins thus produced are subjected to a depilation or unhairing process, usually involving treatment with milk of lime, which conditions the hair and epidermis, and also the fatty tissues on the under side of the skin, so they are readily removed from the skin by mechanical methods. The unhaired skins may be subjected to the bathing and pickling process for enhancing softness and pliability, and are actually converted to leather by tumbling in a box or drum containing tan liquor. After tanning, the leathers are passed into a bath for fixing the tannin, and are then dyed in lukewarm dye baths with mechanical working by means of a tumbler or paddle-wheel after first going through a series of mechanical operations. The leather thus produced, after drying and staking, frequently has a total area considerably less than that of the hide from which it was produced, and the proportionate decrease of total area is termed the "shrinkage" of the hide.

The quantity of leather produced is frequently measured in terms of the total square footage or area of leather, per dozen skins produced, and an undesirably high shrinkage is often observed in customary tannery practice. It is accordingly an important object of this invention to provide means for minimizing the extent of such shrinkage, preserving however the high quality of the leather produced.

Frequently unfinished leather produced in accordance with conventional methods is subjected to an operation wherein a mixture of oils and tanning materials is worked into the pores of the leather by rolling or tumbling in a drum. By reason of the presence of these added materials the thickness of the leather is increased but the aforementioned operation tends to break down the skin and to decrease its tensile strength. It is accordingly another object of the invention to eliminate such operations, and to produce leather having high tensile strength consistent with thickness and minimum shrinkage.

In conventional tannery operations the hides and skins are necessarily subjected to the action

2

of various treating liquids for rather long periods of time. Various attempts to speed the tanning, coloring, and liming operations by increasing strength or temperature of treating liquids or chemicals have usually resulted in the production of inferior leather. Accordingly it is a still further object of this invention to provide an apparatus and process for producing high quality leather in a minimum time, and at greatly decreased cost as compared to prevailing practice.

Other and further objects and advantages of the invention, including the simplicity of the same and the ease with which it may be carried into effect in combination with existing tannery operations, will appear in further detail hereinafter.

In summary, the invention concerns method and means for producing leather from skins, wherein the skins are subjected to the action of high vacuum and are then contacted with leather treating chemicals while held under said high vacuum.

25

*Unhairing*

The skins, which have been cured and are normally received at the tannery in substantially dehydrated form, are sorted, weighed and loaded directly into a rotary vacuum drum, without preliminary soaking. This rotary vacuum drum has a plurality of radially disposed inwardly directed pegs arranged circumferentially on its inner race for rotation with the drum, which serve to lift the skins and then to drop them as the drum is rotated. The drum is also fitted with suitable conduits and attachments whereby it may be evacuated. Care is taken during the skin-loading operation to avoid packing, or in other words it is important to load the skins loosely into the drum. The drum door is then closed to form an air-tight seal and the air is exhausted slowly from the drum by means of a vacuum pump. Vacuum readings for the vacuum within the drum are preferably taken periodically, say every ten to fifteen minutes, for example. When a vacuum of about 15 millimeters is attained, the drum is rotated very slowly, at intervals of about one-half hour, for example at a rate of 18-20 revolutions per minute, for a total of four to six revolutions for each half-hour period. The skins are thus lifted by the pegs, flexed, and then dropped as the drum rotates. It is found that further rotation at this stage may tend to crack or damage the skins to an undesirable extent, while proper evacuation

is difficult if not impossible to achieve in a minimum time without rotation to tumble the skins when the vacuum present has reached a value in the vicinity of 15 mm. Hg.

Evacuation is continued until a high vacuum equivalent to an absolute pressure of 2000-500 microns Hg is attained within the drum. Such high vacuum is then held for a period of about 30-60 minutes and the vacuum connections to the pump are sealed off. Lining chemicals in the form of a homogeneous liquid or milk, at a temperature of about 85° F., are admitted to the drum. During the course of lime introduction the vacuum drum is stationary. The lime is desirably a relatively dilute solution or suspension and preferably consists essentially of about 30% calcium oxide, 2% caustic soda or soda ash, and 1-2½% depilatory such as sodium sulfate, dimethylamine sulfate, or the composition commercially known as Sebacol, for example, the foregoing percentages being by weight and based upon the total weight of dry skins present for treatment. Sebacol is a powder comprising a mixture of sodium sulfite, sodium bisulfite, and caustic lime.

Upon admission of the lime and complete coverage of skins by the lime solution or milk, the drum is rotated for a time under the vacuum remaining in the sealed drum, preferably for 5 minutes to one hour. This step is important, the time of rotation varying with the type skins being processed. The vacuum is then broken while drum rotation is continued by admitting air to the drum, and this is followed by further drum rotation at the same speed for about one-half to one hour. The drum is then opened and the skins are inspected for softness, pliability, and degree of lime penetration.

By reason of the processing in accordance with the invention, the skins are rendered soft and pliable within an unusually short period of time, on the order of approximately one-half to one hour. Treatment in accordance with this invention eliminates the clear water soak and liming operation heretofore found necessary, in one short operation. Frequently periods of at least two days have been required, in practicing conventional processes, merely for soaking alone.

Completeness of lime penetration is determined by cutting a skin, preferably along the backbone, which is usually most difficult to penetrate, and dropping a standard phenolphthalein solution on the skin cross section thus exposed. Dark red coloration due to phenolphthalein action on lime solution indicates the extent of lime penetration while light pink coloration will appear, usually just under the grain surface of the skin section, not reached by penetration of full strength lime solution. By reason of treatment in accordance with this invention, excellent lime penetration is attained in the surprisingly short time of ½-1 hour, as indicated.

The skins are now permitted to soak in the remaining lime at atmospheric pressure for a period of about 22-24 hours, with drum rotation for at least 10-15 minutes during each four-hour period. Drum rotation at this point is important. The agitation stirs the lime suspension preventing settling, and also flexes the skins periodically working fresh lime into the skins.

Following the lime soak at atmospheric pressure, water is introduced into the drum, gradually diluting the lime. The dilute lime is then run out of the drum and the skins are washed with circulating fresh water at 85-90° F. They are now ready for beaming.

Skins such as goat skins and the like, treated in accordance with this invention, are thus prepared for beaming in an unusually short time. Moreover, they are submerged or in contact with liquid for an unusually short time, and surprisingly show a square footage gain, or at least show a marked shrinkage decrease as compared to similar skins subjected to the conventional water soak and liming treatment.

#### Coloring

The coloring process of the present invention is broadly applicable for treating leather whether or not the leather has been beamed or tanned, or beamed and tanned in accordance with the high vacuum process previously set forth herein. The skins may be beamed or limed, unhairied, fleshed, tanned, delimed, bated, pickled and pearly in the usual manner preparatory to coloring in accordance with the process of this invention. The pieces of leather to be colored are loaded individually into the drum, which is then closed. Vacuum is applied in the manner indicated in the foregoing description relating to liming, and a vacuum of 2000-500 microns Hg is thus applied to the contents of the drum. Coloring solution consisting essentially of 0.5-5% by weight sulfonated oil per hundred pounds crusted weight of skins, and about 15-30% by weight of basic or direct or acid dye being introduced, based on the total crusted weight of leather stock under treatment. For coloring with black dyes the sulfonated oil is preferably sulfonated marine oil such as cod oil, sperm oil or the like. Ordinarily sulfonated oil and basic color dyes form undesirable precipitates interfering with proper leather coloring but we have found that these ingredients of the basic coloring composition are compatible in the coloring process of this invention. Ordinarily the basic dye would penetrate the leather independently of the sulfonated oil which would merely remain in the form of a separate film on the surface of the leather; even if the oil should be first applied to the leather, thereby effecting penetration, the subsequent application of basic color dyes would throw the sulfonated oil back out of the leather with similar, highly undesirable, results.

Preferably the sulfonated oil and basic dye are introduced as a mixture into the vacuum drum, although other procedures may also be followed. These may, if found desirable in connection with the particular coloring process at hand, be followed by introduction of chrome, aniline, acid and direct dyes, and formic acid into the drum while maintaining the resulting vacuum. Formic acid is introduced into the drum after the introduction of the dyes. Drum rotation is continued during all color admission steps.

Following the introduction of the dyes, the drum rotation is continued for about 5 to 10 minutes, under the remaining vacuum. Air is admitted into the rotating drum while the drum is rotated, rotation is continued at atmospheric pressure for a short period, and the drum is opened for inspection of skins.

The leather is inspected for dye penetration by cutting and examining a cross section of the leather. Ordinarily complete penetration of the entire cross section of the leather piece is not required, but it is important that the extent of penetration be uniform throughout the piece. Accordingly the presence of a white streak disposed substantially just beneath the grain surface, bordered at both sides by uniform deeply

colored strips, is indicative of highly effective and uniform dye penetration. This sort of dye penetration is attained, in unusually short time, by means of the process according to our invention. Moreover the dyed leather has good layout, has proper feel and lies flat without surface wrinkles. Due to the uniformity and completeness of dye absorption little or no excess dye is found on the leather surface.

*Tanning*

Leather may be produced from skins in accordance with the invention by tanning in a manner substantially the same as the previously described coloring process, substituting tan liquor for the specified coloring chemicals. The skins may be tanned whether or not they have been beamed or limed in accordance with this invention, and the advantages of minimum shrinkage, and minimum time required for retaining the skins in the tan liquor, are achieved in either case.

In all the foregoing specific examples of the invention the skins were charged into a rotary vacuum vessel provided with means for raising individual skins out of the liquid and subsequently permitting them to drop into the liquor, meanwhile flexing the skins. While such means are preferably in the form of short pegs disposed at spaced intervals on the inner circumference of a rotating drum, it will be appreciated that equivalent means including paddle-wheels, tumblers, or the like, may be provided for carrying out the steps of the method. It is highly important to remove the skins from the liquid, flex the skins in vacuum, and re-deposit them into the liquid since otherwise the important advantages heretofore pointed out are not realized to the fullest extent. The skins are preferably redeposited by dropping them and permitting free fall through a vertical drop of 4-6 feet or more, causing the skins to strike the surface of the liquid with considerable impact.

It will be appreciated that, while a high vacuum in the range of 2000-500 microns is preferred, it is within the scope of this invention to utilize a high vacuum of about this quantity, provided adequate processing is attained without sacrificing the advantages of improved shrinkage results.

It will further be appreciated that certain features of the invention may be used independently of the use of other features, that equivalent steps and elements may be substituted for the steps and elements specifically referred to, and that reversals and other changes in the sequence of steps of the method may be made, all within the spirit and scope of the invention as defined in the appended claims.

Having thus described our invention, we claim:

1. In a method of processing skins with minimum shrinkage with a solution selected from

- the group consisting of unhairing, tanning and coloring solutions, the steps which comprise charging the skins into an air-tight container, withdrawing air from said container while slowly rotating said container, continuing the air withdrawal until a high vacuum of about 2000-500 microns mercury is attained, introducing said solution into said container to a level substantially covering said skins, and slowly rotating the container lifting the skins above the liquid level, flexing said skins in the evacuated space above the liquid level, and returning said skins below the surface of the liquid while maintaining vacuum in said container.
- 15 2. The method defined in claim 1 wherein the solution is an unhairing solution.
3. The method defined in claim 1 wherein the solution is a tanning solution.
4. The method defined in claim 1 wherein the solution is a coloring solution.
- 20 5. The method defined in claim 4 wherein the coloring solution consists essentially of about 0.5-5% by weight sulphonated oil and 15-30% by weight basic dye.
- 25 6. The method defined in claim 5 wherein the sulfonated oil is a sulfonated marine oil selected from the group consisting of cod oil and sperm oil.
7. The method defined in claim 1 wherein said 30 returning step comprises dropping said skins through a substantial distance causing them to fall solely under the influence of gravity whereby they strike the surface of the solution with considerable impact.
- 35 8. The method defined in claim 7 wherein said skins are caused to fall a distance of at least about four feet.

CHARLES F. RUTHERFORD.  
SAMUEL CAMERON TEASE.  
HARRY LA RUE TROXELL, JR.

References Cited in the file of this patent

UNITED STATES PATENTS

| Number    | Name    | Date          |
|-----------|---------|---------------|
| 1,065,168 | Nance   | June 17, 1913 |
| 1,230,667 | Carr    | June 19, 1917 |
| 1,338,307 | Krouse  | Apr. 27, 1920 |
| 1,789,629 | Kannel  | Jan. 20, 1931 |
| 1,887,972 | Wrangle | Nov. 15, 1932 |
| 2,354,200 | Cutler  | July 25, 1944 |
| 2,438,150 | Cutler  | Mar. 23, 1948 |

FOREIGN PATENTS

| Number  | Country       | Date          |
|---------|---------------|---------------|
| 26,040  | Great Britain | A. D. 1909    |
| 118,155 | Australia     | Mar. 2, 1944  |
| 167,785 | Great Britain | Aug. 15, 1921 |

OTHER REFERENCES

- 60 Wilson, "Modern Practice in Leather Manufacturing," pages 337 and 709, published 1941 by Rheinhold Publishing Company, New York city.